

# UNITED STATES PATENT OFFICE.

FORD M. CLAPP, OF CLEVELAND, OHIO, ASSIGNOR TO THE OHIO VARNISH COMPANY, OF CLEVELAND, OHIO, A CORPORATION OF OHIO.

## GRAINING COMPOUND.

No. 909,847.

Specification of Letters Patent.

Patented Jan. 12, 1909.

Original application filed June 23, 1906, Serial No. 323,032. Divided and this application filed September 4, 1906. Serial No. 333,183.

To all whom it may concern:

Be it known that I, FORD M. CLAPP, a citizen of the United States, residing at Cleveland, in the county of Cuyahoga and State of Ohio, have invented a certain new and useful Improvement in Graining Compounds, of which the following is a full, clear, and exact description.

In graining wood with a graining tool it has heretofore been customary to take a graining pigment varying in color with the different kind of wood to be represented, this pigment being in a dry form and when used being diluted with vinegar or stale beer, or some similar reducer. This has always been inconvenient. The beer or vinegar has a sour, unpleasant odor; is liable to ferment; the dilution must be made at the time of use, and the amount of dilution varies the color, with the result that frequently various parts of the same grained floor present a different appearance. Graining colors in the form of paste, thinned with drier and turpentine or benzin have been used, but they are not adapted for application by a graining tool and require considerable skill in their use.

I have devised a graining compound which may be kept in stock ready mixed for use and may be applied by a graining tool without requiring any special skill on the part of the user.

The present invention relates to the graining compound itself, the process of applying it being covered in my application No. 323,032 filed June 23rd, 1906, of which this application is a division.

I make the pigment of my graining compound of substantially equal portions of raw sienna and whiting. These are mixed together and ground in water sufficient to make a thin paste. This paste is then diluted with alcohol to the proper consistency for use. It is then put up in glass jars and may be preserved indefinitely.

In applying the grainer, I first apply a ground coat of light straw color. After this is dry the graining compound is applied. This is a light yellow color and when dry is hardly perceptible on the light ground, presenting the appearance simply of streaks thereon. With a colored transparent varnish applied to it, however, it gives a beautiful, natural grain to the wood. The tint of this varnish depends on the wood it is intended to imitate;—yellow for oak, brown for walnut, red for cherry, etc. In each case the same graining compound may be used.

One of the advantages of my system is that there need be no special skill on the part of the user, as with ordinary graining. There is no mixing or thinning of the materials; it is simply necessary to apply them with brushes and a graining tool.

The alcohol in the compound not only insures rapid drying, but prevents creeping so that the graining pigment retains its form when it dries. This pigment does not adhere like paint, but is retained in place by the varnish over it.

I claim:

1. A graining compound in fluid form consisting of a pigment ground in water and contained ready for use in alcohol as a vehicle.

2. The composition of matter ready mixed for graining consisting of substantially equal parts of raw sienna and whiting ground in water to make a thin paste and thinned with alcohol in colorless form to make the proper consistency.

In testimony whereof, I hereunto affix my signature in the presence of two witnesses.

FORD M. CLAPP.

Witnesses:

S. E. FOUTS,  
J. B. HULL.